

## UNITED STATES PATENT OFFICE

RICHARD SCHMIDT, OF DESSAU IN ANHALT, GERMANY, ASSIGNOR TO AGFA ANSOC CORPORATION, OF BINGHAMTON, NEW YORK, A CORPORATION OF NEW YORK

MANUFACTURE OF MATERIAL SUITABLE FOR RECEIVING WRITINGS BY ELECTRODECOMPOSITION

No Drawing. Application filed October 15, 1929, Serial No. 399,883, and in Germany October 16, 1928.

The present invention relates to a process of manufacturing material suitable of receiving writings by electro-decomposition; more particularly it relates to a process of impregnating a suitable support with a specific solution of heavy metal salts and to the material obtainable by that process.

If paper, a textile fabric or another suitable support is treated with heavy metal salts capable of forming a sulfide and with a salt which by cathodic reduction evolves hydrogen sulfide, is brought in contact with a current-conducting electrode, a heavy metal sulfide is produced at the point of contact. Colored characters can thus be produced upon the paper. The papers, textile fabrics, or the like, impregnated according to the hitherto known processes of this kind, possess, however, no sufficient stability. Moreover, the impregnating liquors hitherto used are stable only for a short time.

I found, that materials capable of receiving writings by electro-decomposition and of excellent stability can be prepared by impregnating paper, a textile fabric or another suitable support with a weakly acid aqueous solution of double salts of heavy metal salts with alkalinmetal thiosulfate or sodium sulfite. Preferably, I may use for the said purpose a photographic acid fixing bath solution which has already been used. The said used fixing bath solutions contain probably silver double salts of the formula

$[\text{Ag}(\text{S}_2\text{O}_3)]\text{Na}$  or  $[\text{Ag}_2(\text{S}_2\text{O}_3)_3]\text{Na}_4$ , and a solution of a silver halide in alkali bisulfite. The material treated with such a solution is then dried in a current of hot air. The extraordinary stability of the papers or the like thus prepared is due to the acid reaction of the impregnating solution applied. The new impregnating solution remains unaltered for several weeks. By the action of the electric current a precipitate of silver sulfide is produced in the paper.

As the impregnating liquor to be utilized in the new process is a solution which has already been used as a fixing bath in a photographic process, namely a waste product, the costs of the preparation of papers, textile

fabrics, or the like to be electrolytically written on are very much reduced. The process can be rendered still cheaper by recovering the silver from the said fixing bath solution before impregnating the paper with the solution. For this purpose there is added in known manner an excess of finely subdivided metal which is not a precious metal like silver, for instance lead. If fixing baths thus treated and filtered off are used for impregnating paper or the like the precipitate produced on the paper by the electric current consists of the sulfide of the metal used for the precipitation of the silver.

What I claim is:—

1. The process of manufacturing material for receiving writings by electrolytic decomposition which consists in impregnating a support with an acid aqueous solution containing a thiosulfate of the group consisting of an alkalinmetal thiosulfate and ammonium thiosulfate, and a heavy metal salt capable of forming a double salt with said thiosulfates, and drying the material.

2. The process of manufacturing material for receiving writings by electrolytic decomposition which consists in impregnating a support with an acid fixing bath comprising a thiosulfate of the group consisting of an alkalinmetal thiosulfate and ammonium thiosulfate, and an alkalinmetal bisulfite, said fixing bath having already been used in the photographic process, and drying the material.

3. The process which comprises treating an acid fixing bath comprising a thiosulfate of the group consisting of an alkalinmetal thiosulfate and ammonium thiosulfate, and sodium bisulfate, said fixing bath having already been used in the photographic process, with a heavy metal capable of forming a double salt with said thiosulfates in finely subdivided form, filtering off the solution thus obtained, impregnating a support with said filtered off solution, and drying said impregnated support.

4. The process which comprises treating an acid fixing bath comprising a thiosulfate of the group consisting of an alkalinmetal thiosulfate and ammonium thiosulfate, and

sodium bisulfite, said fixing bath having already been used in the photographic process, with lead in finely subdivided form, filtering off the solution thus obtained, impregnating a support with said filtered off solution, and drying said impregnated support.

5. A material capable of receiving writ-

ings by electrolytic decomposition consisting of a support impregnated with a double salt of a thiosulfate of the group consisting of an alkalinmetal thiosulfate and ammonium thiosulfate and a heavy metal salt capable of forming a double salt with said thiosulfates.

RICHARD SCHMIDT.

10

75

15

80

20

85

25

90

30

95

35

100

40

105

45

110

50

115

55

120

60

125

61

130